

## UNITED STATES PATENT OFFICE

2,347,527

## CRACKING OF HYDROCARBONS

Byron M. Vanderbilt, Cranford, N. J., assignor to  
Standard Oil Development Company, a corpora-  
tion of Delaware

No Drawing. Application December 27, 1940,  
Serial No. 372,007

3 Claims. (Cl. 260—680)

The present invention relates to improvements in the art of treating hydrocarbons, and, more particularly, it relates to pretreatment of the inner surfaces of tubes, conduits, and the like, with which the hot reaction vapors contact, for the purpose of inhibiting or reducing the tendency of the metallic substance of the tube from causing excessive coke deposition.

It is well known that in the pyrolysis of hydrocarbons in ferrous and other metallic equipment more coke or carbon is formed and deposited on the inner surfaces of the equipment than when the equipment is constructed from glass or silica. It has been shown, for example, that when 2-butene was cracked to form butadiene, using KA2S alloy tubes to form the cracking coil, the deposition of carbon was copious and soon plugged the reactor so that it was necessary to discontinue the operation in order to remove the coke or carbon. When this equipment was replaced by quartz equipment, the deposition of carbon on the equipment was greatly reduced. My explanation as to why the deposition of carbon is excessive on certain ferrous alloys such as KA2S is that it contains metals which oxidize, and the oxides of these metals act as active catalysts in the decomposition of hydrocarbons which they contact at cracking conditions.

I propose to pretreat metallic equipment, such as cracking coils, with an acid having an ionization constant greater than  $10^{-6}$ , whereupon the equipment is rendered substantially passive toward causing the formation of excessive quantities of coke when subsequently employed in the cracking operation. I prefer to use an aqueous solution of such an acid, but gaseous acidic substances, such as hydrogen chloride, hydrogen iodide, hydrogen bromide, acetic acid, nitric acid, oxides of nitrogen, sulfur dioxide, or sulfur trioxide either in pure form or mixed with inert gases such as nitrogen or admixed with steam or water vapor, may also be employed. The treatment is advantageously carried out at ordinary temperatures, but if the acid is applied in gaseous form a sufficiently high temperature must be employed to keep it vaporized, or at temperatures up to 875° F.

It is also advantageous to combine the action of an acid and a reducing agent for rendering ferrous and ferrous alloy tubes less catalytic toward hydrocarbons. This may be accomplished, for example, by first carrying out the acid treatment followed by treatment with hydrogen at elevated temperatures. Or, the order may be reversed, or, if desired, they may be combined by

5 using a mixture of hydrogen chloride and hydro-  
gen at elevated temperatures, or an aqueous acid  
solution containing an active metal such as zinc  
or tin may be employed at ordinary or slightly  
elevated temperatures.

I have found that metallic tubes to be used in  
the cracking process should be treated with the  
acids or their anhydrides for a period of from  
one minute to several hours, depending upon the  
type and concentration of the agent used. When  
the treatment is discontinued, the hydrocarbon  
oil or vapors undergoing cracking may be then  
passed through the pretreated tubes or other  
equipment.

10 15 20 25 30 35 40 45 50 55 60 65 70 75 80 85 90 95  
The following are concrete examples illustrating  
my invention, but they are set forth with the  
understanding that they do not constitute a re-  
striction or limitation of my invention:

*Example 1*

A series of test runs were carried out by a  
standardized procedure and in special equipment  
designed to give a semi-quantitative measure of  
carbon deposition during the cracking of butene-2 to butadiene in the presence of a metallic  
surface. In these tests the cracking zone con-  
sisted of the annular space between an inner  
KA2S steel tube (18 inches long by  $\frac{1}{2}$  inch out-  
side diameter, and closed at both ends) and an  
outer quartz tube (36 inches long by  $\frac{3}{8}$  inch  
inside diameter) heated in an electrical furnace  
with a 13 inch heating zone. This type of crack-  
ing zone was used in these tests so that com-  
parative results could be obtained quickly and so  
that the metal surface (the outside surface of  
the inner closed metal tube) of the cracking  
zone could be easily inspected and cleaned be-  
tween tests. The quartz tube was also cleaned  
between each test. After the clean reaction zone  
was given a chosen pretreatment, it was flushed  
with nitrogen gas and the cracking reaction test  
run was carried out by feeding 2-butene at a  
constant flow rate of 25 cc./sec. and at a furnace  
temperature of 867° C., giving a gas temperature  
of about 830° C. and a contact time (time of resi-  
dence in the cracking zone) of 0.015 second. The  
flow of 2-butene was usually maintained for about  
10 minutes, except in the cases where the reac-  
tion zone became plugged with carbon in a much  
shorter time. Since the annular reaction zone  
was only approximately  $\frac{1}{64}$  inch in radius, carbon  
deposition was immediately detectable by an in-  
crease in resistance to flow of the butene feed,  
as measured by a mercury manometer at the  
entry end of the furnace. The normal operating

pressure with a similar all-quartz reaction zone of the same size was about 25 mm. of mercury. With the above described metal-quartz reaction zone, lack of any pretreatment of the reaction zone resulted in a rapid build-up of the line pressure during the cracking reaction. When the pressure reached 80 mm. of hydrogen, the annular zone was considered to be plugged.

Employing the above equipment and procedure, a series of runs was made on the cracking of 2-butene in the reaction zone following various pretreating methods for making the KA2S steel tube less catalytic toward carbon deposition, the rate of pressure increase while maintaining a constant butene flow rate being taken as a measure of the rate of carbon deposition. The following table gives the pretreatments used and the results obtained:

| Test | Method of pretreating the KA2S steel tube                                                                                                 | Effect on cracking of 2-butene                                       |                                                                |
|------|-------------------------------------------------------------------------------------------------------------------------------------------|----------------------------------------------------------------------|----------------------------------------------------------------|
|      |                                                                                                                                           | Time required to plug reaction zone                                  | Nature of carbon deposit                                       |
| A    | Mechanical clearing with brush or suitable scraper                                                                                        | 1½ min.                                                              | Copious and fairly coherent.                                   |
| B    | NH <sub>3</sub> passed over cleaned tube at rate of 10 cc./sec. for 1½ hrs. at 500° C.                                                    | 2 min.                                                               | Do.                                                            |
| C    | H <sub>2</sub> S passed over cleaned tube at rate of 10 cc./sec. for 1½ hrs. at 600°-700° C.                                              | 3½ min.                                                              | Hard layer, but scaled off easily.                             |
| D    | Cleaned tube treated with 25% NaOH at 95° C. for ½ hr.                                                                                    | 1 min.                                                               | Copious layer, scaled off easily.                              |
| E    | Cleaned tube treated with fused NaOH at 500° C. for 1½ hrs. and washed with dilute acetic acid and with water.                            | 6 min.                                                               | Very sooty.                                                    |
| F    | Carbon deposit burned out by passing air through reaction zone at 700°-740° C. for ½ hr.                                                  | 1½ min.                                                              | Very copious layer and much soot carried out of zone by gases. |
| G    | Excess of carbon deposit removed mechanically and then air passed through reaction zone at 700°-820° C. for ½ hr.                         | 1½ min.                                                              | Do.                                                            |
| H    | Cleaned tube treated with 10% acetic acid by weight for 2 hrs. at room temperature.                                                       | Only 5 mm. pressure increase in 9 min.                               | Thin uniform coating.                                          |
| I    | Cleaned tube treated with 2 normal HNO <sub>3</sub> for 2 min. at room temperature and washed with water.                                 | 7 mm. pressure increase in 5 min. but no further increase in 23 min. | Small and coherent layer.                                      |
| J    | Carbon burned out with air at 530°-650° C. for 45 min. followed by treatment with SO <sub>2</sub> at 675°-830° C. for 45 min.             | 15 mm. pressure increase in 10 min.                                  | Quite hard layer, peeled off easily.                           |
| K    | Mechanically cleaned tube treated with SO <sub>2</sub> at 640°-810° C. for 40 min. followed by H <sub>2</sub> at 840°-870° C. for 10 min. | 3 mm. pressure increase in 6 min.                                    | Very small layer, peeled off easily.                           |

### Example 2

An all-metal cracking zone consisting of the annular space between two KA2S steel tubes, one (18 inches long by 11/32 inch outside diameter and closed at both ends) fitting inside the other (36 inches long by 5/8 inch inside diameter), was pretreated with 0.2 normal HNO<sub>3</sub> for 20 minutes at room temperature, washed with water, dried, and treated with hydrogen at 770°-845° C. for 25 minutes. 2-butene was then fed at a rate of 25 cc./second to the cracking zone which was maintained at a furnace temperature of about 860° C., giving a gas cracking temperature of about 820° C. and a contact time of 0.015 second. A run of 22 minutes duration was made with a line pressure increase of only 9 mm. of hydrogen during this period. At the completion of the run, a very small coherent layer of carbon was found in the heated portion of the reaction zone. In this experiment a 57.1% conversion of the 2-butene was obtained with a 30.3% yield of butadiene based on butene converted. This compares very well with the 30.5% yield which is obtained at the same conversion in all-quartz equipment.

Although the above tests were carried out with KA2S steel tubes, while other steel alloys such as NCT-3 (25% Cr, 20% Ni, 0.15% C, and the balance Fe.) or Ascoloy-55 (26%-30% Cr, 1% Mn, 0.6% Ni, and the balance Fe.) etc. may be more applicable for the construction of reaction zones for high temperature cracking, the results obtained will likewise apply to the other steel alloys since iron is believed to be the chief of-

fender as regards promotion of carbon deposition.

In view of my tests, I have found that one highly desirable method for pretreating a cracking coil to be used in the thermal cracking of hydrocarbons involves the following:

Before firing the furnace in which the tubes are disposed, the inside of the tubes should be contacted for about one-half hour with an acid having an ionization constant greater than 10<sup>-6</sup>, such, as for example, 2% nitric acid, followed by washing with water. Thereafter methane or hydrogen at atmospheric or higher pressure should be kept in the cracking tubes while bringing them to cracking temperature. When necessary to shut down the cracking coil, hydrogen or methane should be kept in the tubes while cooling and air should be excluded from con-

tact with the interior of the cracking tubes until they are cold. Decoking of the tubes should be by mechanical means, avoiding burning out with air. Hydrogen is preferably passed through the cracking tubes at the operating temperature for one-half to one hour after each shutdown prior to the introduction of the feed stock. If, at any time, the carbon deposit appears to be excessive, the tubes may be cooled, the excess carbon removed mechanically, and the tubes pretreated by one of the methods described above.

It will be distinctly understood that the precise details hereinbefore enumerated are purely illustrative of my invention and many modifications of it may be made without departing from the spirit thereof, which invention is based on the proposition that alloys which are used in the construction of cracking coil tubes may, and often do, contain metals which catalyze the decomposition of hydrocarbons, so that when hydrocarbons are passed through them in a liquid or gaseous phase they cause the deposition of excessive amounts of coke which necessitates frequent shutdowns to remove the said coke. I have found that this tendency of ferrous metals and ferrous alloys with manganese, nickel, chromium, and the like, to catalyze the hydrocarbon decomposition and to thereby cause excessive coke deposition can be greatly minimized by treating the insides of the tubes with an acid having an ionization constant greater than 10<sup>-6</sup>, employing also, if desired, or necessary, a treatment with hydrogen as hereinbefore set forth.

What I claim is:

1. In a process for effecting pyrolysis of gase-

ous hydrocarbons in metallic apparatus, the effectiveness of which becomes reduced during the course of the operation, the steps which comprise interrupting the pyrolysis treatment when the effectiveness of such apparatus becomes thus reduced, removing carbonaceous deposits from the metal surfaces, thereafter treating said metal surfaces with an acidic substance having an ionization constant greater than  $10^{-6}$ , thereafter treating said metal surfaces with hydrogen, and reemploying the apparatus for the pyrolysis of said gases.

2. In a process for effecting pyrolysis of hydrocarbons in metallic apparatus, the effectiveness of which becomes reduced during the course of the operation, the method of treating said metal surfaces to reduce coke deposition thereon which comprises treating said metal surfaces with an acidic substance having an ionization constant greater than  $10^{-6}$ , thereafter washing 20

said metal surfaces to remove the acidic substances retained thereon, and subsequently treating the metal surfaces with hydrogen prior to contacting the same with said gaseous hydrocarbons to be pyrolyzed.

3. In a process for effecting pyrolysis of gaseous hydrocarbons wherein said gaseous hydrocarbons are contacted with metal surfaces at relatively high temperatures and wherein carbonaceous deposits tend to form on said metal surfaces under operating temperature conditions, the method of reducing the amount of carbonaceous deposits formed on said surfaces which comprises initially contacting said surfaces with an acidic substance having an ionization constant greater than  $10^{-6}$  and continuously maintaining an atmosphere of hydrogen in contact with said metal surfaces.

BYRON M. VANDERBILT.